

# UNITED STATES PATENT OFFICE.

JAMES THOMAS RHYNE, OF DURANT, MISSISSIPPI, ASSIGNOR TO HIMSELF AND WILLIAM CALVIN RED, OF SAME PLACE, AND JOSEPH PETERS, OF FORT SCOTT, KANSAS.

## TANNING PROCESS.

SPECIFICATION forming part of Letters Patent No. 351,204, dated October 19, 1886.

Application filed May 5, 1886. Serial No. 201,221. (No specimens.)

*To all whom it may concern:*

Be it known that I, JAMES THOMAS RHYNE, of Durant, in the county of Holmes and State of Mississippi, have invented a new and useful Improvement in Tanning and Stuffing Leather, of which the following is a full, clear, and exact description.

This invention is designed as an improvement upon the process as described in Letters Patent No. 128,246, for compounds used in treating the leather, granted to Joseph Peters June 25, 1872; but it differs in the proportions of the ingredients up to the period when the leather or hide is taken from the vats, and is especially different in the finishing of the leather—that is, in the whole treatment of it after removal of the leather or hide from the vats.

The invention is not only applicable to the tanning, &c., of hides for making leather of a superior quality for different purposes in less time, &c., but it may also be used to advantage by farmers and others in the tanning of hides, furs, and skins of many kinds without having resort to expensive or special appliances, as it can be mainly done in barrels or hogsheads. It will suffice here, however, to describe the invention as used for tanning and finishing or stuffing leather, and among the advantages secured may be named the following:

In the first place, by my improved process, substantially as hereinabove described, the tanning can be successfully carried on in all countries or places, inasmuch as no bark is required; and in countries or places where bark is not a natural product it is expensive to import said material, besides which bark-tanning requires more time. In the next place, less labor is required to handle and work the same amount of hides or leather. Again, all grades or kinds of leather can be made or tanned, including firm and good sole-leather; also superior harness, shoe, glove, and belting leathers and lacing, or what is commonly known as "whang-leather," saddle-skirtings, and in fact all kinds and qualities whatever, as well as furs. The apparatus used is or may be the same as that used in ordinary tanning and stuffing operations. Consequently there is no necessity here either to show or describe it in detail.

The invention consists in certain treatments of the hide or skin and in the use of certain hot mixtures or compounds to the grain and flesh sides of the hide, essentially as herein-after described, and pointed out in the claim. 55

The following description will explain in full how my invention is carried into practice.

I first soak the hide in clear water until it is soft enough to shave off the glaze or flinty flesh with a light-edged currying-knife. This 60 preliminary treatment is important, and results in a large saving of mechanical labor and quickens the softening, liming, and tanning parts of the process. The hide after being thus shaved is then thrown back into 65 the pool or receptacle of clear water, where it is allowed to remain about ten (10) or twelve (12) hours, more or less—that is, long enough to perfectly soften the hide, which result is expedited by the currying operation 70 above named. The hide is then taken out of the clear water a second time and thrown onto the ordinary or any suitable breaking-beam, flesh side up, and run over with a fleshing-knife. This completes the hide ready for 75 liming, as usual in tanning, the formula I prefer to adopt being about one (1) bushel of slaked lime to fifty (50) gallons of soft water; but other proportions may be used as the strength of the preparation is recruited by the 80 addition from time to time of more lime. After this, the hide is rinsed by throwing it a third time into the pool or receptacle of clear water, and then taken to a smooth flat table and with a steel sleek the hair worked off, 85 which is much more expeditiously done than on a fleshing-beam. The hide thus prepared is again rinsed off in any suitable vessel and again thrown into a pool or body of clean soft water, and raised once a day, or thereabout, 90 until bated low enough to work the lime out. This can be ascertained by pinching up the grain between the thumb and forefinger. After this the hide is taken back to the scouring-table and sleeked off on the flesh side and 95 turned over and stoned until the lime is thoroughly expressed, and subsequently rinsed in clear water, when it is ready for immersion in the tanning-liquor.

The tanning-liquor is prepared as follows: 100

To eight (8) gallons of water I add about three (3) pounds of salt, half ( $\frac{1}{2}$ ) of a pound of salt-peter, ten (10) pounds of gambia, after which I add, by agitation, sulphuric acid, one (1) pound. The hides are placed in this liquor, which is strengthened as it becomes weak by adding the above-named ingredients in their respective proportions, or thereabout, and are handled two or three times a day for the first 5 to two or three days, and afterward once a day. After the tan has been struck about half through, then the hides are thrown up in pile to drain, and afterward beamed, or in lieu thereof passed through the press-rollers, well 10 on flesh side, which hastens the tanning. They 15 are then thrown back into the tanning-liquor, and the process of beaming, if necessary, repeated to hasten the tanning. After the tan has thoroughly struck through, the hides are 20 removed from the tanning-liquor.

The next proceeding is to immerse the hides in lye, instead of brushing them with lye, as in Peters' process, and to use a lye of the following strength, viz: the contents of one box, 25 equal to about one (1) pound of concentrated lye, dissolved in twenty (20) gallons (more or less) of soft, clean water, allowing the hides to remain from thirty to sixty minutes. This serves to thoroughly neutralize the acids.

30 Each hide is then thrown into clean soft water and permitted to remain from twenty to forty hours, according to the thickness of the hide. This soaks out the remaining particles of the tanning chemicals, which, if not removed, 35 would attack and injure the leather and impair its durability. Upon removing the hide from the clear water it is placed on a table, with its flesh side up, and sleeked and brushed to remove all remaining ooze. The grain side 40 of the hide is treated by stoning and brushing, frequently pouring on clean water during this operation to prevent the leather from staining. The hide is then hung in the shade until it ceases to drip, after which tanning-oil, 45 boiling hot, is poured on the grain side and brushed in thoroughly. This method of applying the oil preserves the leather, causes it to penetrate more perfectly, and makes the leather more pliant.

50 After ten or twelve hours of the above treatment, I apply to the flesh side of the hide a boiling hot mixture composed of one (1) part tar, one (1) part tallow, and two (2) parts of tanners' oil, brushing the same in thoroughly.

55 After which the hide is hung up in the shade to dry. This treatment causes the tar and

tallow to fill up the pores, rendering the leather water-proof.

In these last two steps it should be observed that the mixtures applied to the grain and 60 flesh sides are used boiling hot, instead of applying the oil and dubbing, as heretofore, in a cold state. By applying the mixtures hot they are driven into the pores of the leather, thus solidifying the leather and rendering it 65 impervious to water. By applying the mixture to the grain side hot, too, it is only necessary to wait ten or twelve hours before applying the mixture to the flesh side, instead of having to wait four or five days as when 70 the treatment is a cold one, and no lye, which rots the leather, is used in these two treatments with the hot mixtures.

75 After the leather has been thus prepared all surface grease is washed off with common bar soap and the surface blackened with ink, as in what is known as "oak-tanning leather"—that is, thus treated on the grain side when the leather is to be used for harness purposes, or is required to be blackened on the grain side. 80 Other leather to be blackened on the flesh side is differently treated.

Having thus fully described my invention, I claim as new and desire to secure by Letters Patent—

85 My improvement in tanning and finishing hides, which consists in the following steps, to wit: first, soaking the hide in clear water; second, removing all gristly or flinty flesh; third, again soaking the hide in fresh water; 90 fourth, beaming and liming; fifth, again soaking in fresh water; sixth, unhairing on a smooth flat table with a steel sleek; seventh, removing lime by thoroughly soaking in water and stoning; eighth, tanning with a mixture composed of water, gambia, salt, sulphuric acid, and saltpeter; ninth, beaming by hand or passing through pressure-rollers; tenth, immersing thoroughly in lye-water and using a light-edge currying-knife on flesh side 100 and again placing in fresh water; eleventh, taking out the hides and hanging in the shade until dry, and treating to boiling-hot tanner's oil (fish-oil and beeswax) on grain side, and applying to the flesh side a boiling mixture 105 of tar, tallow, and tanner's oil, (fish-oil and beeswax,) and finally coloring in the usual manner, substantially as above stated.

JAMES THOMAS RHYNE.

Witnesses:

D. S. SHLENKER,  
J. M. DYER.